

## 1

3,093,585

**ESTER BASE LUBRICANT COMPOSITIONS**  
 Hans Low and William W. Reynolds, East Alton, Ill., and  
 Donald W. Schmulling, St. Louis, Mo., assignors to  
 Shell Oil Company, New York, N.Y., a corporation of  
 Delaware  
 No Drawing. Filed June 6, 1960, Ser. No. 33,952  
 10 Claims. (Cl. 252—37.2)

This invention relates to a lubricant composition containing a superior antioxidant combination. More particularly, the present invention relates to an additive combination for ester base lubricant compositions having excellent stabilizing effects at extremely high lubricating temperatures.

One of the greatest problems in lubricating at high temperatures is to develop a composition which will not easily oxidize to form acidic components which in turn cause harmful deposits or sludges in the composition. This problem is especially difficult to overcome when dealing with high temperatures such as encountered in modern aircraft gas turbine engines and hydraulic systems where hot areas in the range of from 350–750° F. are contacted by the lubricant.

It is an object of the present invention to provide improved ester compositions. It is a particular object of the invention to provide ester compositions having reduced tendencies to form acidic oxidation products. It is a particular object of the invention to provide ester lubricants especially useful as gas turbine lubricants and hydraulic fluids.

Now, in accordance with the present invention, a superior lubricant composition is provided comprising an ester-type base fluid and oxidation stabilizing amounts of both an amine of the group consisting of certain triazines and certain pyridylamines in combination with critically limited proportions of complexes of such classes of amines with copper salts of fatty acids. In one aspect of the invention provision is made for partially oxidizing the amines to be used in the formation of such copper salt complexes. The optimum mol ratio of the combination is from 2 to 75 mols of total amine for each mol of copper.

The copper complexes which are formed between the amine and the copper salt are believed to be of the "square planar" type. However, the precise structure of the complexes has not been absolutely determined. They appear to exist in a ratio of about 2 mols of the amine for each mol of the copper salt. Part of the unexpected character of the present invention lies in the fact that copper is known to be a serious accelerator of oxidation. Consequently the present invention is based upon the discovery that an optimum ratio exists wherein an excess of free amine is present beyond the amount necessary for forming the complex for the copper salt and within which ratio a remarkable stabilization of the oxidation properties of the ester base lubricant is observed.

The copper salts to be employed in the preparation of the subject complexes are preferably those with the copper in the second oxidative state (copper II), while the fatty acid radical may be derived from any fatty acid having from 2–24 carbon atoms. These include the usual acids such as acetic, propionic, butyric, hexoic, octanoic, dodecanoic, capric, caprylic, caproic, stearic, oleic, linoleic, etc. It is preferred that the acid be saturated and have from 2 to 12 carbon atoms per molecule.

## 2

The amines which are utilized in their free form and also in complex with the copper salt are of two general categories. These may be referred to as pyridylamines and triazines. The pyridylamines are those having at least one pyridyl radical and preferably two and comprise unsubstituted pyridylamines as well as alkyl substituted, and those pyridylamines having as substituent groups amino radicals, aryl radicals, aminoaryls, aminoalkyls, and triazyl radicals. Table A, which follows, lists typical pyridylamines coming within the scope of this invention.

TABLE A

## Pyridylamines

|    |                                        |
|----|----------------------------------------|
|    | Monopyridylamines:                     |
| 15 | 2-pyridylamine                         |
|    | 3-pyridylamine                         |
|    | Dipyridylamines:                       |
| 20 | 2,2'-dipyridylamine                    |
|    | 2,3'-dipyridylamine                    |
|    | 2,4'-dipyridylamine                    |
|    | 3,3'-dipyridylamine                    |
|    | 4,4'-dipyridylamine                    |
|    | Alkylpyridylamines:                    |
| 25 | 2,2'-di(4-ethylpyridyl)amine           |
|    | 4,4'-di(2-tert-butylpyridyl)amine      |
|    | 2-pyridyl-2'-(4-isopropylpyridyl)amine |
|    | Aminopyridylamines:                    |
| 30 | 2-tolyl-2'-(4-aminopyridyl)amine       |
|    | 2,2'-(3-N-ethylaminopyridyl)amine      |
|    | Arylpyridylamines:                     |
| 35 | (2-pyridyl)(2'-benzyl)amine            |
|    | (4-pyridyl)(2'-phenyl)amine            |
|    | (2-pyridyl)(2'-naphthyl)amine          |
|    | (2-pyridyl)(2-triazyl)amine            |

The triazines may be used as the sole amine in the composition or may be combined with the pyridylamines. Suitable types are those constituted by unsubstituted triazine, or more preferably the guanamines in addition to monoaminotriazines, alkyltriazines, aryltriazines or triazinylamine. Table B which follows lists typical species suitable for this purpose.

TABLE B

## Triazines

|    |                                          |
|----|------------------------------------------|
|    | Guanamines:                              |
| 50 | 2,4-diamino-6-benzyl-triazine            |
|    | 2,4-diamino-6-methyl triazine            |
|    | 2,4-diamino-6-propyl triazine            |
|    | 2,4-diamino-triazine                     |
| 55 | 1-N-ethyl-2,4-diamino triazine           |
|    | 1-N-phenyl-2,4-diamino triazine          |
|    | 2,3-di-(N-ethyl)-2,4-diamino triazine    |
|    | 1,3,5-tri(N-methyl)-2,4-diamino triazine |
|    | 2,4-diamino-6-phenyl-triazine            |
|    | Monoamino triazines:                     |
| 60 | 2-(N-methylamino)-triazine               |
|    | 2-(N-phenylamino)-triazine               |
|    | 2-amino-triazine                         |
|    | Alkyl triazines:                         |
| 65 | 2,4-diethyltriazine                      |
|    | 2,4,6-trimethyl triazine                 |
|    | 2-methyl-4,6-diethyl triazine            |
|    | 2-methyl-4-amino triazine                |

## Aryl triazines:

- 2,4-diphenyl-triazine  
2-phenyl-4-amino-triazine  
2-benzyl-triazine  
2-benzyl-4(N-benzylamino)triazine

## Triazinylamines:

- Triazinylamine  
(triazinyl)(phenyl)amine  
(triazinyl)(2-pyridyl)amine  
di(triazinyl)amine

The copper salt complexes of these amine types may be formed in situ or may be preformed before dispersal in the ester base lubricants. The complexes are immediately formed by combining solutions such as alcohol solutions of the amine and copper salt and evaporating to dryness. However, complexes appear to be just as efficiently formed by combining the free amine and the copper salt in the ester lubricant.

While the structure of the complex has not been finalized, it is believed to be represented in a specific instance as according to the following diagram:



The formation of metal complex is an equilibrium reaction; therefore, an excess of free amine appears to serve two principal purposes. First, it minimizes the amount of free soluble copper ion which would act as a pro-oxidant and secondly it assures as large an amount of active inhibitor as possible by displacing the equilibrium toward the product, namely, the complex. If excessive amounts of the copper compound are present, then the pro-oxidant effect of copper becomes predominant and causes an acceleration rather than a retardation of oxidation. On the other hand, if excessive amounts of free amine are present (or not enough copper to form sufficient amounts of the complex, the active inhibitor) then the oxidation inhibition is minimized since the free amines do not appear to be very effective inhibitors. Thus, it was found by means of comparative testing that the maximum oxidation inhibition was obtained when the mol ratio of total amine to copper was between about 2 and about 75, preferably between about 5 and about 35.

The mixtures of free amines and copper complexes are found to be effective in aliphatic esters which are used primarily for synthetic hydraulic fluids and gas turbine lubricants as well as for other associated purposes. Broadly, the principal classes included within this broad class of aliphatic esters comprise esters formed between dicarboxylic acids and monohydric alcohols; esters formed between neopentyl glycols and monohydric alcohols; esters of pentaerythritol or its dimers with monohydric alcohols; and the so-called "complex esters" which constitute various combinations of dibasic acids, glycols and alcohols or dibasic acids, glycols and nonobasic acids. Table C outlines the various alternative structures contemplated as "complex esters" as well as listing briefly typical starting materials for the formation of such esters.

TABLE C

## Complex esters (By ester-forming components):

- Alcohol-(dibasic acid-glycol)-monobasic acid  
 $R_1-(OOCR_2COO-R_3)_n-OOCR_4$   
 See U.S. 2,575,195  
 Alcohol-dibasic acid-(glycol-dibasic acid)<sub>n</sub>-alcohol



See U.S. 2,703,811  
Monobasic acid-glycol-(dibasic acid-glycol)<sub>n</sub> monobasic acid



See U.S. 2,575,196

## Monohydric alcohols:

- 2-ethylbutyl alcohol  
2-ethylhexyl alcohol

## 10 Monobasic acids:

- Caproic acids  
Pelargonic acid  
Capric acid

## Glycols:

- 15 Neopentyl glycol  
Ethylene glycol  
Propylene glycol

## Dibasic acids:

- 20 Sebacic acid  
Azelaic acid

As diesters there may be used one or more of the compounds of the formula  $ROOC-Z-COOR$  wherein Z is an alkylene chain of four to eight carbon atoms and R is an alkyl group of four to fourteen carbon atoms, being the residue of an aliphatic monohydric alcohol from butyl to tetradecyl alcohols. Dicarboxylic acids which provide the above esters are adipic, pimelic, suberic, azelaic, and sebacic. The alcohols include butyl, iso-

butyl, or sec-butyl alcohols and the various amyl, hexyl, octyl, nonyl, decyl, undecyl, dodecyl, and tetradecyl alcohols. The alcohols with branched hydrocarbon chains provide diesters with particularly desirable properties. Typical of these are isobutyl, 2-ethylbutyl, 2-ethylhexyl, 1-methylhexyl, 1-methylheptyl, 1-methyl-4-ethyloctyl, 2,2,4-trimethylhexyl, 2-isopropyl-3,3-dimethylbutyl, 1,4-dimethylbutyl, and 1-isobutyl-4-ethyloctyl alcohols.

## Ester Lubes

- 40 bis(2-ethylhexyl)sebacate  
bis(isononyl)sebacate  
bis(2-ethylhexyl)adipate  
bis(1-methylheptyl)azelate  
bis(2,2,4-trimethylhexyl)pimelate  
bis(1,4-diethylhexyl)adipate  
45 bis(1,4-dimethyloctyl)adipate  
bis(2-ethylbutyl)suberate  
(2-ethylhexyl)(isononyl)sebacate  
(1-methylhexyl)(2-ethylbutyl)sebacate

50 The aliphatic polyesters which may be utilized as the lubricating fluids are preferably tetraesters, such as the pentaerythritol esters or the dimers or trimers of the same. Preferably, each radical contains from 4 to 18 carbon atoms each and preferably from 6 to 14 carbon atoms each. Typical species include pentaerythritol tetracaprate, dipentaerythritol hexavalerate, pentaerythritol tetraheptoate, pentaerythritol dicaproate divalerate, pentaerythritol tricaproate heptoate and mixtures thereof. It will be noted that the esters may be either mixed esters or mixtures of homo esters, the best rheological properties being obtained with mixed esters and with mixtures of esters. For use at elevated temperatures the dipentaerythritol esters are preferred due to their greater molecular weight and consequently higher boiling points.

65 The course of oxidation as indicated by the rate of oxygen absorption in the composition of this invention indicates that the amine in complex form with the copper salt is oxidized prior to its assuming its intended function of acting as an oxidation inhibitor. The oxidation of the amine may take place prior to or subsequent to incorporation of the amine in the ester base lubricant. Consequently, the invention will be understood to include the use of not only the amines per se but also their oxidation products as well as the copper complexes of such oxidized products. The exact nature of the oxidation

product has not been elucidated; however, the fraction of the oxidized product found to be most active in the prevention of oxidation of the ester base lubricant has a nitrogen-to-copper molar ratio in the order of about 20-30, while the less effective fractions of the oxidized product have nitrogen-to-copper molar ratios in the order of 3-6.

Still further and unexpected reductions in oxidation of the ester base lubricant are obtained by the additional presence of certain phenolic compounds, particularly alkylene bisphenols. Such compounds are preferably those typified by the following structure:

## METHYLENE BISPHENOLS



The phenolic compounds may be modified by the presence of alkyl radicals on one or both of the phenolic nuclei. Typical compounds are as follows:

- 4,4'-methylenebis(2,6-di-tertiary-butylphenol)  
4,4'-methylenebis(2-(2-ethylhexyl)phenol)  
2,2'-methylenebis(4-isopropylphenol)

The data contained in the working examples will illustrate the benefits obtained by the use of such bisphenols in addition to the combination of the copper complex and free amines as described hereinbefore. The following examples illustrate the use of this invention.

## EXAMPLE I

*Preparation of a copper complex between copper octoate and a triazine.*—An alcoholic solution of copper (II) octoate was mixed with an alcoholic solution of 2,4-diamino-6-phenyl-1,3,5-triazine(benzoguanamine). The green precipitate has a melting point of 210-214° C. and an elemental analysis showing that it contains 55.4 percent by weight of carbon, 7.42 percent hydrogen, 13.3 percent nitrogen and 14.0 percent copper. This agrees with the postulated formula



However, the experimentally determined molecular weight was 945, almost twice as much as the empirical formula and indicates the likelihood of dimerization. This is more plausible since it enables the copper (II) to form a square planar complex.

## EXAMPLE II

*Preparation of a copper salt complex with a dipyridylamine.*—Copper (II) acetate and 2,2'-dipyridylamine were mixed in an alcoholic solution and evaporated to dryness. Analysis of the product gave an empirical formula of  $(\text{C}_{10}\text{H}_9\text{N}_3)_2 \cdot (\text{Cu})(\text{C}_2\text{H}_3\text{O}_2)_2$ . Accordingly, one molecule of copper (II) acetate forms a planar complex with two molecules of the bidentate ligand dipyridylamine. The complex contains 17.5 percent copper and 11 percent nitrogen.

## EXAMPLE III

*Oxidation inhibition of a mixed pentaerythritol ester.*—A pentaerythritol ester of a mixture of fatty acids averaging  $\text{C}_8\text{-C}_{10}$  per ester linkage was modified with 0.025 mol of 2,2-dipyridylamine (22-DPA) and with other

inhibitors as listed in Table 1 below. The various compositions listed were tested by heating at 400° F. with oxygen being bubbled through the sample at the rate of 1 liter of air per hour.

TABLE 1

|    | Inhibitor, 0.025 M                   | Catalyst <sup>1</sup> | Oxidation time, hours |
|----|--------------------------------------|-----------------------|-----------------------|
| 10 | None                                 | None                  | 14                    |
|    | None                                 | Cu, Fe, Ag, Al        | 12                    |
|    | Phenothiazine                        | None                  | 37                    |
|    | Do                                   | Cu, Fe, Ag, Al        | 52                    |
|    | 4,4'-methylenebis (diterbutylphenol) | None                  | 27                    |
|    | Do                                   | Cu, Fe, Ag, Al        | 24                    |
| 15 | 2,2'-dipyridylamine                  | None                  | 16                    |
|    | Do                                   | Cu, Fe, Ag, Al        | 48                    |
|    | 22-DPA/Cu acetate complex            | None                  | 92                    |
|    | Do                                   | Cu, Fe, Ag, Al        | 68                    |
|    | Copper octoate                       | None                  | 16                    |

<sup>1</sup>Metal washers.

- 20 It will be seen by reference to the above table that the unmodified base fluid oxidized to the arbitrary limit set in about 14 hours (the arbitrary limit is that time required for the absorption of 1.0 millimole of oxygen per gram of base fluid). The table also shows that the use of a well-known antioxidant, phenothiazine, resulted in extending this oxidation time (OT) to 37 hours. A standard phenolic inhibitor was not as effective as the latter. It is significant to note that 2,2'-dipyridylamine had essentially no oxidation inhibiting effect. Copper octoate also exhibits substantially no oxidation inhibiting activity when utilized in the absence of an amine of the present invention. However, it is significant to note that when a mixture of 2,2'-dipyridylamine and the copper acetate complex are mixed in the same base lubricant 35 highly effective oxidation inhibition is obtained. Similar formulations wherein the metal catalysts (metal washers of copper, iron, silver and aluminum) are replaced by a soluble copper salt exhibit the same inhibitory effect in the several compositions tested.

- 30 An investigation of the effect of mol ratio of free amine to copper complex was made employing the same pentaerythritol ester containing 0.025 mol of 2,2'-dipyridylamine to which was added varying proportions of copper octoate. 45 Table 2 which follows shows the data obtained in this respect and indicates that the optimum oxidation inhibition is obtained with molar ratios of free amine to copper between about 2 and about 75. The data given in the middle column of this table reflects the total amine versus 50 copper salt. Since the copper takes up two mols of amine per mole of copper salt, the free amine is the net of the total amine minus 2.

TABLE 2

| Copper octoate, in ppm. Cu <sup>+</sup> | Molar ratio, total Amine/Cu | OT, hours |
|-----------------------------------------|-----------------------------|-----------|
| 0                                       | 438                         | 16        |
| 3.3                                     | 73.0                        | 75        |
| 20                                      | 29.1                        | 143       |
| 50                                      | 13.2                        | 160       |
| 110                                     | 7.65                        | 155       |
| 190                                     | 3.82                        | 145       |
| 380                                     | 1.91                        | 92        |
| 760                                     | 0.96                        | 35        |
| 1,520                                   |                             | 16        |

## EXAMPLE IV

70 The pentaerythritol ester base fluid was modified with 0.025 mol of benzoguanamine per liter of solution. The table which follows shows the effect upon oxidation inhibition of adding copper octoate to this composition. Copper octoate added in this manner forms a complex with 75 a part of the amine in situ.

TABLE 3

| Copper octoate in p.p.m. Cu <sup>+2</sup> | Molar ratio total Amine/Cu | OT, hours |
|-------------------------------------------|----------------------------|-----------|
| 0                                         | 438                        | 15        |
| 3.3                                       | 73.0                       | 44        |
| 20                                        | 29.1                       | 62        |
| 50                                        | 13.2                       | 83        |
| 110                                       | 7.65                       | 85        |
| 190                                       | 3.82                       | 89        |
| 380                                       | 1.91                       | 47        |
| 760                                       | 0.96                       | 33        |
| 1,520                                     |                            |           |

## EXAMPLE V

*Oil properties of oxidized oil.*—Table 4 which follows shows the benefits gained by the use of a combination of benzoguanamine (BG) with varying amounts of copper catalyst. It is noteworthy that within the claimed molar ratio the acid number of the oxidized oil is at a minimum, thus indicating that the peroxide production was also minimized by this combination.

TABLE 4

| Amine 0.025 M | Metal                        | Molar ratio, amine/copper | OT, hours | Acid No. |
|---------------|------------------------------|---------------------------|-----------|----------|
| None          | Solid Cu                     |                           | 14        | 5.1      |
| None          | 50 p.p.m. Cu <sup>+2</sup> * |                           | 16        | 5.9      |
| BG            | 180 p.p.m. Cu <sup>+2</sup>  | 7.6                       | 85        | 4.2      |
| BG            | 760 p.p.m. Cu <sup>+2</sup>  | 1.9                       | 47        | 5.1      |

\*Added as copper octoate.

## EXAMPLE VI

*Co-additive effect with a methylene bisphenol.*—Similar compositions were modified with a typical bisphenol namely 4,4-methylene bis(2,4-di-tertiarybutylphenol). It will be seen according to the data which follows that an unexpected coadditive effect is obtained by the presence of this bisphenol in addition to the copper complex and an excess of a free amine.

TABLE 5

| No. | Additive, 0.025 M                             | OT, hours | OT-14 <sup>1</sup> | (OT-14) Comb. (OT-14) <sup>2</sup> |
|-----|-----------------------------------------------|-----------|--------------------|------------------------------------|
| 1   | None                                          | 14        |                    |                                    |
| 2   | Benzoguanamine                                | 15        | 1                  |                                    |
| 3   | 4,4'-methylenebis(2,4-di-tertiarybutylphenol) | 27        | 13                 |                                    |
| 4   | Cu octoate, 50 p.p.m. Cu <sup>+2</sup>        | 16        | 2                  |                                    |
| 5   | (2)+(4)                                       | 62        | 48                 | +45                                |
| 6   | (3)+(4)                                       | 24        | 10                 | -5                                 |
| 7   | (2)+(3)+(4)                                   | 91        | 77                 | +61                                |

<sup>1</sup> Net OT, due to additive alone, i.e., after deduction of the hours of OT by the base stock alone (14 hours).

<sup>2</sup> The difference between the hours obtained experimentally (e.g., 48 for blend No. 5) and the sum of the number of hours in the same column, attained with the individual inhibitors (e.g., 1+2 for blends No. 2 and 4).

## EXAMPLE VII

*Preparation of oxidized 2,2-dipyridylamine and its copper complex.*—To 10 g. of 2,2-dipyridylamine in a 100 ml. round-bottom flask was added 15 ml. glacial acetic acid. The solution was heated for 1 hour at 190° C. mantle temperature. After cooling to room temperature, 20 ml. of 30 percent hydrogen peroxide was added and the liquid temperature raised to 70° C. for 1 hour and 80° C. for 2 hours. An additional 5 ml. of 30 percent hydroperoxide were added and the temperature raised to 90° C. for 1 hour. To half of this solution was added 3.4 g. of copper acetate monohydrate and the solution boiled to a semisolid. This was stored in a vacuum desiccator for 4 days with Drierite and sodium hydroxide pellets.

The above material was separated into 4 fractions by solvent extraction. The first portion was insoluble in ethanol, M.P. >400° C. Dilution of the alcohol solution with water gave a water insoluble second fraction, 5 M.P. 132–135° C. The third portion was a precipitate obtained by adding ether to an ethanol solution of fraction 2, M.P. 181–192° C. The filtrate of fraction 3 gave fraction 4 on evaporation of solvent; it was a dark green viscous liquid and was ether, water and ethanol soluble.

10 The analysis of each fraction and effect on oxidation follow:

| Fraction | Percent N | Percent Cu | N/Cu mol ratio | OT, hours |
|----------|-----------|------------|----------------|-----------|
| 15       |           |            |                |           |
| 1        | 13.6      | 20.2       | 3.1            | 13        |
| 2        | 15.7      | 17.0       | 4.2            | 31        |
| 3        | 15.8      | 12.0       | 6.0            | 37        |
| 4        | 19.5      | 3.52       | 25.1           | 46        |

20 We claim as our invention:

1. A synthetic ester base lubricant composition comprising a major proportion of a pentaerythritol tetraester of a fatty acid and minor oxidation-inhibiting proportions each of benzoguanamine and a copper octoate complex 25 with benzoguanamine, the mol ratio of total amine to copper being between about 5 and about 35.

2. A synthetic ester base lubricant composition comprising a major proportion of a pentaerythritol tetraester of a fatty acid and minor oxidation-inhibiting proportions 30 each of 2,2'-dipyridylamine and a copper diacetate complex with 2,2'-dipyridylamine, the mol ratio of total amine to copper being between about 5 and about 35.

3. A synthetic ester base lubricant composition comprising a major proportion of a pentaerythritol tetraester 35 of a fatty acid and minor oxidation-inhibiting proportions each of an arylaminotriazine and a copper complex of a copper C<sub>2</sub>–24 fatty acid salt with a triazine, the mol ratio of total amine to copper being between about 5 and about 35.

4. A synthetic ester base lubricant composition comprising a major proportion of a pentaerythritol tetraester of a fatty acid and minor oxidation-inhibiting proportions 40 each of 2,2'-dipyridylamine and a copper dioctoate complex with 2,2'-dipyridylamine, the mol ratio of total amine to copper being between about 5 and about 35.

5. A synthetic ester base lubricant composition comprising a major proportion of a pentaerythritol tetraester of a fatty acid and minor oxidation-inhibiting proportions 45 each of 2,2'-dipyridylamine and a copper C<sub>2</sub>–24 fatty acid salt complex with 2,2'-dipyridylamine, the mol ratio of total amine to copper being between about 5 and about 35.

6. A synthetic ester base lubricant composition comprising a major proportion of a pentaerythritol ester of an aliphatic monocarboxylic acid and minor oxidation-inhibiting amounts each of a diaminotriazine and a copper C<sub>2</sub>–24 fatty acid salt complex with a pyridylamine, the mol ratio of total amine to copper being between about 2 and about 75.

7. A synthetic ester base lubricant composition comprising a major proportion of a pentaerythritol ester and minor oxidation-inhibiting amounts each of a triazine and a copper C<sub>2</sub>–24 fatty acid salt complex, with a pyridylamine, the mol ratio of total amine to copper being between about 2 and about 75.

8. A synthetic ester base lubricant composition comprising a major proportion of a pentaerythritol ester and minor oxidation-inhibiting amounts each of a pyridylamine and a copper C<sub>2</sub>–24 fatty acid salt complex with a pyridylamine, the mol ratio of total amine to copper being between about 2 and about 75.

9. A synthetic ester base lubricant composition comprising a major proportion of a pentaerythritol ester of an aliphatic monocarboxylic acid and minor oxidation-inhibiting amounts each of a dipyridylamine and a copper

$C_2$ -24 fatty acid salt complex with a pyridylamine, the mol ratio of total amine to copper being between about 2 and about 75.

10. A synthetic ester base lubricant composition comprising a major proportion of an aliphatic ester of an aliphatic carboxylic acid and minor oxidation-inhibiting amounts each of a copper  $C_2$ -24 fatty acid salt complex of an amine of the group consisting of pyridylamines, aminotriazines and mixtures thereof and a free amine of the same group, the mol ratio of total amine to copper being between about 2 and about 75.

## References Cited in the file of this patent

## UNITED STATES PATENTS

|           |                     |               |
|-----------|---------------------|---------------|
| 2,961,406 | McNeil -----        | Nov. 22, 1960 |
| 2,962,439 | Lauer -----         | Nov. 29, 1960 |
| 2,976,238 | Elliot et al. ----- | Mar. 21, 1961 |

## OTHER REFERENCES

Atkins et al.: "I. and E. Chem.", vol. 39, No. 4, April 1957, pp. 491-493.

10 Barnes et al.: "Lubrication Engineering," August 1957, pp. 454-458.